

## UNITED STATES PATENT OFFICE

1,948,246

## METAL ROLL

William H. Seaman, Hammond, Ind.

No Drawing. Application October 2, 1930  
Serial No. 486,042

9 Claims. (Cl. 80—58)

The present invention relates in general to a novel alloy of iron for use in a chilled cast iron roll employed for rolling metal articles and in particular to a chilled iron alloy roll having a "chill" or "a definite chill" as it is sometimes called.

5 One of the objects of the present invention is to provide an alloy iron of such character that the hardness of the working depth or chill may be increased.

10 Another object is to provide a novel alloy of iron in which the toughness of the working depth or chill may be increased.

15 Another object is to provide an iron alloy which when cast in chilled roll will increase the amount of work that may be done with it before it is dressed.

20 A further object is to provide a novel iron alloy which is easier handled in casting in a chilled mold and which will give more uniform characteristics.

25 Still another object is to provide a novel iron alloy which is particularly beneficial in obtaining an iron alloy roll that may be substituted for a forged steel roll and which will give better results in such cases.

30 There are other objects of my invention which, together with the foregoing, will be described in the detailed specification which is to follow:

I have ascertained that the addition of molybdenum to a large number of alloys, having as 35 modifying constituents, carbon, manganese, silicon, sulphur, phosphorus, chromium and nickel, has a very advantageous effect in that with the modifying ingredients properly proportioned for any particularly desired work it will greatly increase its hardness and toughness and that the 40 alloy, when cast in a chilled mold, will provide a roll that wears better and has longer life.

The quantity of the product that may be turned out by such a roll is greatly increased before the 45 roll has to again be dressed, and the alloy itself is easier to handle in casting. Further, an alloy of more uniform character is obtained in this manner. The proportion of molybdenum with the various other modifying elements mentioned 50 is given below and may be proportioned to give alloys of varying characteristics in a manner well understood by those skilled in the art

forms its well known function of tending to control the hardness, the nickel also having a hardening effect.

It is to be pointed out that the alloys generally are somewhat similar in character to those disclosed in my co-pending application, Serial No. 449,686, filed May 3, 1930, with the addition of molybdenum. In fact, alloys having the same proportion of modifying constituents as disclosed in my co-pending application cited above, may be employed with the addition of molybdenum between .15% and .5% to give a greater degree of hardness, toughness and improved wearing qualities, whereby the roll is better adapted to perform where high sclerescopic hardness is necessary, as 75 in the instances set forth in said co-pending application.

My aforesaid other application Serial No. 449,686, contains the following table of hardnesses and ingredients to secure the same.

|            | T.C.               | Mn               | Si                | S                  | P                | Cr               | Ni                 |    |
|------------|--------------------|------------------|-------------------|--------------------|------------------|------------------|--------------------|----|
| 70 to 80.  | 2.60<br>to<br>3.15 | .24<br>to<br>.27 | .55<br>to<br>.65  | .100<br>to<br>.115 | .18<br>to<br>.50 | .20<br>to<br>.30 | 2.50<br>to<br>3.00 | 85 |
| 80 to 90.  | 3.15<br>to<br>3.20 | .15<br>to<br>.22 | .25<br>to<br>.35  | .115<br>to<br>.130 | .18<br>to<br>.60 | .25<br>to<br>.35 | 3.00<br>to<br>4.00 | 70 |
| 90 to 100. | 3.25<br>to<br>.20  | .15<br>to<br>.25 | .15<br>to<br>.150 | .120<br>to<br>.50  | .18<br>to<br>.35 | .25<br>to<br>.35 | 4.00<br>to<br>5.00 | 75 |

My invention may be variously modified without departing from the spirit and scope thereof, as set forth in the appended claims.

I claim:

1. A cast iron alloy chilled roll, the alloy including as modifying elements carbon from 2.60% to 3.35%, manganese .10% to .40%, chromium .15% to .65%, nickel 1.25% to 5.00%, and 100 molybdenum in substantially the same proportion as the chromium.

2. A cast iron alloy chilled roll, the alloy including as modifying elements carbon from 2.60% to 3.35%, manganese .10% to .40%, silicon .20% to 1.00%, chromium .15% to .65%, nickel 1.25% to 5.00%, and molybdenum .15% to .50%.

3. A cast iron alloy chilled roll, the alloy including as modifying elements carbon from 2.60% to 3.35%, manganese .10% to .40%, silicon .20% to 1.00%, sulphur .05% to .200%, chromium .15% to .65%, nickel 1.25% to 5.00%, and molybdenum .15% to 50%.

4. A cast iron alloy chilled roll, the alloy including as modifying elements carbon from 2.60% to 3.35%, manganese .10% to .40%, silicon .20% to 1.00%, sulphur .05% to .200%, phosphorus .05% to .55%, chromium .15% to .65%, nickel 1.25% to 5.00%, and molybdenum .15% to .50%.

| 50 | T.C.               | Mn               | Si                | S                | P                | Cr               | Ni                 | Mo               |
|----|--------------------|------------------|-------------------|------------------|------------------|------------------|--------------------|------------------|
|    | 2.60<br>to<br>3.35 | .10<br>to<br>.40 | .20<br>to<br>1.00 | .05<br>to<br>.20 | .05<br>to<br>.55 | .15<br>to<br>.65 | 1.25<br>to<br>5.00 | .15<br>to<br>.50 |
|    |                    |                  |                   |                  |                  |                  |                    |                  |

55 with the addition of sufficient iron to make up 100% in each instance.

It will be seen that the amount of molybdenum is quite similar to the amount of chromium. The molybdenum content increases the toughness and 60 hardness of the chill. The carbon, of course, per-

5. A cast iron alloy chilled roll, the alloy including as modifying elements total carbon 2.60% to 3.35%, silicon .20% to 1.00%, chromium .15% to .65%, nickel 1.25% to 5.00%, and molybdenum in substantially the same proportion as chromium. 85
6. A high carbon cast iron alloy roll having a chilled wearing surface and having nickel and chromium for increasing the depth of the chill in the proportion of nickel from 1.25% to 5.00% 10 and chromium in the proportion of .15% to .65% and having molybdenum for increasing the toughness and hardness of the wearing surface in the proportion of .15% to .50%. 90
7. A chilled iron alloy roll having a definite chill and containing a hardening and toughening agent such as carbon and nickel, in an amount within certain limits to produce a desired degree of hardness and toughness, and also containing a chill affecting ingredient such as silicon in 20 amount between certain limits to cooperate with the amount of hardening and toughening agent employed and not to exceed 1.0, and also containing a further hardening agent. 95
8. A chilled iron alloy roll containing a hardening and toughening agent such as carbon and nickel, in amount between certain limits to secure 100

WILLIAM H. SEAMAN. 100

88 105  
 89  
 90 110  
 91  
 92 115  
 93  
 94 120  
 95  
 96 125  
 97  
 98 130  
 99  
 100 135  
 101  
 102 140  
 103  
 104 145  
 105  
 106 150